

# United States Patent

[19]

McCann

[11] 3,815,881

[45] June 11, 1974

[54] TUBE ANNEALING APPARATUS AND METHOD

[75] Inventor: Milton H. McCann, Wheeling, W. Va.

[73] Assignee: Riker Laboratories, Inc., Northridge, Calif.

[22] Filed: Mar. 8, 1973

[21] Appl. No.: 339,357

Related U.S. Application Data

[62] Division of Ser. No. 210,502, Dec. 21, 1971, Pat. No. 3,776,785.

[52] U.S. Cl. .... 266/5 F, 432/230, 432/11, 266/23 Q

[51] Int. Cl. .... C21d 9/08

[58] Field of Search ..... 148/151; 266/23 Q, 23 SF, 432/230, 231, 121, 137

[56] References Cited

UNITED STATES PATENTS

|           |         |         |           |
|-----------|---------|---------|-----------|
| 232,882   | 10/1880 | Bennett | 432/230   |
| 1,605,535 | 11/1926 | Foisy   | 266/5 F X |
| 2,288,008 | 6/1942  | Mason   | 432/230 X |
| 2,795,411 | 6/1957  | Court   | 432/230   |
| 2,907,858 | 10/1959 | Distler | 266/4 X   |

FOREIGN PATENTS OR APPLICATIONS

1,040,578 10/1958 Germany ..... 266/5

Primary Examiner—Roy Lake

Assistant Examiner—Paul A. Bell

Attorney, Agent, or Firm—Parmelee, Miller, Welsh & Kratz

[57] ABSTRACT

An apparatus and method for annealing thin-walled metal tubes which comprise a body portion and a tapered shoulder portion which has a relatively thickened wall. The tubes are disposed upon a transport conveyor which rapidly moves tubes through an annealing furnace wherein a first heat source is disposed for maintaining a uniform high temperature within the chamber, and wherein a second heat source comprising a plurality of combustion flame burners are disposed within the chamber along the path of travel of the conveyor. The flame emanating from the second combustible flame burners is directed upon the shoulder portion of the tubes which are passed through the annealing temperature without rupture or deformation of the thin-walled tubes.

5 Claims, 3 Drawing Figures



PATENTED JUN 11 1974

3,815,881

SHEET 1 OF 2

FIG. 1.



FIG. 2.



PATENTED JUN 11 1974

3,815,881

SHEET 2 OF 2

FIG. 3.



## TUBE ANNEALING APPARATUS AND METHOD

This is a divisional of application Ser. No. 210,502, filed Dec. 21, 1971, now U.S. Pat. 3,776,785.

### BACKGROUND OF THE INVENTION

Tubular metallic containers are widely used as packaging containers in commerce. It is generally desired that the tubular metal container have a low temper to facilitate the consumer's usage. Most such tubular metal containers are formed of aluminum. The containers are formed typically by impact forming a solid disc of aluminum into the thin-walled tubular member. The impact forming step significantly raises the temper of the metal. It has been the practice to anneal the impact formed tubular members at a relatively high temperature for several minutes to render the metal soft and workable. In heating very thin-walled tubes, uneven heating or local overheating can easily result in a rupture of the tube or in distortion of the tube.

Prior art annealing furnaces typically comprise a tube supporting conveyor moving within a convective heating zone furnace within which the tubes are held for at least several minutes to effect the annealing process.

### SUMMARY OF THE INVENTION

An apparatus and method is provided for rapidly bringing the tubular members to the annealing temperature of the metal without rupture or deformation of the thin-walled tubes. The typical thin-walled metal tubes comprise a uniform diameter body portion and a tapered shoulder portion at one end thereof, which has a relatively thickened wall. An enclosed heating chamber is provided with an inlet and an outlet opening, and a tube support and transport conveyor means is disposed to pass into the inlet opening and out of the outlet opening of the annealing chamber. The width of the tube support and transport means is about equal to the body portion of the tube disposed thereon, with the shoulder portion end of the tube extending beyond one side of the conveyor means. A heat source is disposed within the annealing chamber for maintaining a uniform high temperature within the chamber. A plurality of combustion flame burners are disposed within the chamber along the path of travel of the conveyor means, which burners are disposed to direct the flames emanating therefrom upon the shoulder portion of the tubes disposed upon the conveyor means, whereby the tubes are rapidly brought to the annealing temperature.

### BRIEF DESCRIPTION OF THE DRAWINGS

FIG. 1 is a schematic representation of the tube annealing system.

FIG. 2 is a partial plan view of the furnace portion of the tube annealing system.

FIG. 3 is an end view of the furnace of the tube annealing system with end wall removed.

### DESCRIPTION OF THE PREFERRED EMBODIMENTS

The tube annealing system shown schematically in FIG. 1 comprises; the annealing furnace 10 which has an inlet opening 11 at one end thereof, and an outlet opening 12 at the other end thereof. An endless chain conveyor 13 is disposed to pass through the annealing furnace 10 with the return path being beneath the furnace. Tube support means 14 are provided on the con-

veyor 13 and more particularly comprise a plurality of inverted V-shaped supports 15, with the apex of the V transverse to the direction of travel of the conveyor so that tube troughs 16 are formed between adjacent inverted V-shaped supports 15. The inverted V-shaped supports are formed of high temperature resistant metal plates with a plurality of apertures 17 therethrough. Plate burners 18 are disposed within the furnace 10 beneath the conveyor means 13. The plate burners 18 are gas fired and serve to heat the V-shaped supports 15, which have apertures 17 therein whereby the tubes 19 disposed thereon are also heated with a relatively uniform temperature being maintained within the annealing furnace 10. The tubes 19 comprise a relatively uniform diameter body portion 20 which has a uniform very thin wall thickness, for example of the order of about 0.003 to 0.005 inch, and a tapered shoulder portion 21 at one end of the body portion 20. The tapered shoulder portion 21 has a relatively thickened wall, for example about 0.015 to 0.035 inches thick.

A tube feed conveyor means 22 moves the tubes to indexing means 23, which deposits the tubes 19 upon the horizontal annealing conveyor 13 in a tube trough 16. The indexing means 23 also serves to position the tube properly upon the annealing conveyor, with the shoulder portion of the tube projecting beyond the side of the inverted V-shaped supports 15 toward the shoulder burners 24. The individual shoulder burners 24 are connected to a gas supply manifold 25.

The tubes are loaded onto the annealing conveyor 13 from a tube conveyor 22 which deposits the tubes 19 within the tube troughs 16 formed by the V-shaped supports 15. The body portion 20 of tubes 19 fits into troughs 16, with the shoulder portion 21 extending beyond the edge of the V-shaped supports 15. The plurality of combustion flame shoulder burners 24 are disposed from the side wall of the annealing furnace 10 on the same side of the conveyor 13 from which the shoulder portions 21 extend. The shoulder burners 24 are disposed to direct the flame emanating therefrom upon the tapered shoulder portion 21 of respective tubes which are passed through the annealing furnace 10. The tubes passing out the outlet opening 12 from the annealing furnace 10 are deposited into tube holding means 26 mounted upon a cooling tower conveyor 27, which circulates the tubes within the cooling structure 28 to permit determination of the temperature of the tubes before advancing the tubes onto the discharge conveyor 29 which brings the tubes to the next processing station. The structure of the annealing furnace 10 can be seen in greater detail in FIG. 3 wherein the furnace 10 comprises an outer frame 30, inner frame 31 which includes a refractory block upper portion 32, which permits combusted gas to pass slowly upward and out the stack 33. Support means 34 is provided for the conveyor 13, and drive means 35, for the conveyor 13, is generally indicated.

The invention can be best understood by reference to a specific exemplary embodiment wherein the tubes 19 are formed of aluminum with a body portion of about nine inches long with a diameter of about 1 1/2 inch, a wall thickness of about 3 thousandths of an inch, and wherein the shoulder portion extends for about 1 1/2 inches. The shoulder portion has a wall thickness of about 0.030 in. The plate burners 18 heat the high temperature resistant V-shaped supports 15 to a high tem-

perature which permits maintenance of a uniform temperature distribution along the length of the tubes to insure against rupture and deformation of the thin-walled body portion when the shoulder portion is directly heated by the flames from the gas shoulder burners. The flame temperature of the combusted gas at the point where the flames from the shoulder burners impinge the tapered shoulder portion are about 2,400° to 2,600°F.. The flame is preferably directed upon the underside of the tapered shoulder portion. For an annealing furnace which is about 35 inches long, preferably 17 shoulder burners are employed with the first 11 burners starting at the inlet opening being spaced about 1½ inch apart, and with the remaining six burners spaced about 2½ inches apart.

It is possible utilizing the apparatus and method of the present invention to anneal the aluminum tubes described in about 15 seconds. This is a significant reduction in annealing time from the several minutes previously required, and yet the annealing is carried out without destructive rupturing of the very thin-walled tube and without deformation of the tube also.

The temperature of the tubes upon entering the furnace is about 100°F., and in passing through the furnace in about 15 seconds the temperature of the tubes is raised to about 960°F., well above the annealing temperature of the aluminum which is at least about 850°F.

In summary, the present invention permits the rapid annealing of work hardened thin-wall tubes, to provide a soft, workable squeeze tube. Vast numbers of tubes must be so annealed, and the time saving had from the present invention is significant. The annealing is carried out rapidly without deformation or damage to the tubes.

The flame from the shoulder burners as can be seen in FIG. 3 is directed in the same horizontal plane in which the tubes are disposed, with the flame impinging the shoulder portion of the tube as the tube passes through the flame. The movement of the tube through the flame means that the flame is not directed continuously on one portion of the tube shoulder.

The spacing of the shoulder burners results in a succession of rapid heating periods when the flame impinges the moving tube, and conductive heating periods between burners during which the temperature of the tube tends to equalize. The shoulder burners can be more widely spaced at the exit end of the furnace because the tubes have already been raised to the proper annealing temperature, with the latter burners just

10 maintaining the tubes at this temperature.

I claim:

1. Apparatus for annealing thin-walled metal tubes which comprise a body portion and a tapered shoulder portion at one end thereof which has a relatively thickened wall comprising:

a. an enclosed heating chamber having an inlet and an outlet opening;

b. a tube support and transport conveyor means which is disposed to pass into the inlet opening and out of the outlet opening, with the width of the tube support and transport conveyor means being about equal to the body portion of the tube disposed thereon with the shoulder portion end of the tube extending beyond one side of the conveyor means;

c. a heat source disposed within the chamber for maintaining a uniform high temperature within the chamber;

d. a plurality of combustion flame burners disposed within the chamber along the path of travel of the conveyor means, which burners are disposed to direct the flame therefrom upon the shoulder portion of the tubes disposed upon the conveyor means, whereby the tubes are rapidly brought to annealing temperature without rupture or deformation of the thin-walled tubes.

2. The apparatus specified in claim 1, wherein the tube support and conveyor means comprises inverted V-shaped supports with the apex of the V transverse to the direction of travel so that the tube troughs are formed between adjacent inverted V-shaped supports, and wherein the inverted V-shaped supports are formed of a high-temperature resistant metal plates with a plurality of apertures therethrough.

3. The apparatus specified in claim 1, wherein the heat source comprises a plurality of plate burners disposed beneath the conveyor means.

4. The apparatus specified in claim 1, wherein the tubes are impact formed aluminum, and wherein the shoulder portion is exposed to a flame temperature of from 2,400° to 2,600°F. from the combustion flame shoulder burners.

5. The apparatus specified in claim 1, wherein the combustion flame burners are spaced along the length of the heating chamber, said burners being more closely spaced at the entrance end of the heating chamber.

\* \* \* \* \*

UNITED STATES PATENT OFFICE  
CERTIFICATE OF CORRECTION

Patent No. 3,815,881

Dated June 11, 1974

Inventor(s) Milton H. McCann

It is certified that error appears in the above-identified patent and that said Letters Patent are hereby corrected as shown below:

**In Item [73] on the face of the patent, delete as Assignee:**

**"Riker Laboratories, Inc.,  
Northridge, Calif."**

**and insert therefor**

**--Wheeling Stamping Company  
Wheeling, W. Va.--**

Signed and sealed this 5th day of November 1974.

(SEAL)

Attest:

MC COY M. GIBSON JR.  
Attesting Officer

C. MARSHALL DANN  
Commissioner of Patents